

## UNITED STATES PATENT OFFICE

2,398,242

## PAINT AND VARNISH REMOVER

John D. Morgan, South Orange, and Russell E. Lowe, East Orange, N. J., assignors to Cities Service Oil Company, New York, N. Y., a corporation of Pennsylvania

No Drawing. Application October 10, 1944,  
Serial No. 538,082

4 Claims. (Cl. 252—118)

This invention relates to improvements in paint and varnish removing compositions, and is a continuation-in-part of our pending application Serial No. 435,862, filed March 23, 1942.

Many of the commonly used removing compounds are most effective in lifting paint and lacquers from their supporting surfaces only when applied in a heated state. It appears that the heat serves both to speed the penetration of the solvent through the protective coating material, as well as to render it more effective in destroying the bond between the coating and its supporting surface. It is readily evident, however, that the heating of these volatile materials results in great wastage. In order to overcome this difficulty, it is more or less common practice to immerse articles in a bath of the heated solvent, and to limit evaporation losses by the use of vapor recovery equipment.

It is readily evident that the hot dipping process is not practicable for the stripping of paint from articles of any considerable size. It is hardly feasible, for example, to provide dipping tanks and auxiliary handling equipment of sufficient capacity to allow for the treatment of complete aircraft, or even of its major sub-assemblies. In cases of this kind it has sometimes been the practice to brush a hot remover solution over the painted surface, and by repeated operations to maintain a film of the remover on the surface for a long enough time to allow it to lift the paint. This operation is time consuming, wasteful, and not very effective. The thin film of remover evaporates so rapidly that it does not have time to penetrate the protective coating, and the fact that the solution is hot increases this effect. In addition, these light-bodied solvents run off of vertical or sloping surfaces almost as fast as they can be applied, so that a very large part of the remover does not remain in contact with the paint or varnish coating long enough to have any real effect upon it.

It can also be readily appreciated that hot dipping, or even hot brushing, cannot be used in removing paints from articles which would be damaged by the heat of the operation, and furthermore that it is not economically feasible to provide equipment for heating remover solutions in all of the many places where their use is required. By way of illustration, it need hardly be pointed

out that the hot process is utterly impractical at the many aircraft repair fields which are located in the remotest parts of the globe.

The principal object of the invention is to provide a paint and varnish remover which acts effectively at normal atmospheric temperatures to penetrate protective coatings of paint and lacquer, and to loosen them from their supporting surfaces, and which is of such a nature that it may readily be applied with the simplest of equipment that may be found almost anywhere.

It is a further and more specific object of the invention to provide a paint removing composition having the nature of a paste which is soft enough to allow it to be spread readily over a painted surface with a putty knife, or any other convenient tool, and which is stiff and sticky enough to adhere to a painted surface, even when disposed in a vertical position, so that its active solvent ingredients may remain in contact with the paint for a long enough period of time to penetrate and loosen it from the underlying part.

It is a further object of the invention to provide a paint and varnish remover composition of a pasty nature in which the active ingredients are not corrosive to ordinary metals and other materials of construction and which may therefore be retained on the surfaces of articles from which paint is to be removed for relatively long periods of time without giving rise to any danger that the underlying parts will be corroded or damaged. This is particularly important in a remover which is to be used for stripping lacquer from aircraft parts which are most frequently made of aluminum or aluminum alloys, and are of such a nature that even the slightest corrosion cannot be tolerated.

Our preferred remover composition consists of a mixture of the following ingredients in the proportions indicated:

|                   | Percent by volume | Parts by weight |
|-------------------|-------------------|-----------------|
| 45 Water          | 10                | 10.00           |
| Monooctanolamine  | 10                | 10.20           |
| Kerosene          | 20                | 8.20            |
| 1-nitropropane    | 30                | 30.00           |
| Oleic acid        | 10                | 8.95            |
| Isopropyl alcohol | 20                | 15.75           |

In this mixture each part of oleic acid will react with .216 parts of monoethanolamine to form a soap which serves as a carrier for the other ingredients, and the final composition will therefore be substantially as follows:

|                         | Percent by weight | Parts by weight |    |
|-------------------------|-------------------|-----------------|----|
| Water                   | 12.02             | 10.00           | 10 |
| Monoethanolamine        | 9.94              | 8.27            |    |
| Monoethanolamine oleate | 13.00             | 10.89           |    |
| Kerosene                | 9.80              | 8.20            |    |
| 1-nitropropane          | 36.20             | 30.09           |    |
| Isopropyl alcohol       | 18.95             | 15.75           |    |

This product is of paste-like character which is soft enough to permit its application and easy spreading over a painted surface with a putty knife, an ordinary wooden stick, or almost any readily available tool. At the same time it is stiff enough and sufficiently sticky to adhere to a painted surface on the underside of an article, or to a vertical wall, and to stand on that surface for extended periods of time. The material may, for example, be smeared on the fuselage or wings of an aircraft awaiting repair, and will be found to stick to its sides and bottom without any tendency to run off. This is a feature of particular advantage, because it completely overcomes one of the objections to prior art removers, namely, that of difficulty of maintaining a film of the remover on the surface to be stripped.

The composition has proven to be highly effective in penetrating and loosening paints, and particularly lacquers of the kind employed as protective coatings for aircraft. It has been found that the pasty composition holds its solvent ingredients in intimate contact with a painted surface long enough to allow the solvent ingredients to penetrate the protective coating and to loosen its bond with the supporting article. The composition will, for example, completely strip an anodized aluminum alloy panel which has been finished with a primer and enamel top coats, and will leave a surface which is suitable for refinishing without further preparation.

It is of note that the vapor pressure of the composition is very low, so that at normal atmospheric temperatures the several solvents have little or no tendency to pass away as vapors before they can accomplish their functions. Also it will be appreciated that the active ingredients which have been employed, do not give off noxious odors which might constitute either a source of annoyance or a real physical hazard to operators who must apply the composition to articles to be stripped.

A further feature of importance is that none of the ingredients of our composition has any corrosive effect upon aluminum alloys (either polished or anodized surfaces) which are ordinarily used in aircraft, or upon steel, cadmium plated steel, or other common materials of construction. This is a matter of particular importance in a remover such as ours, which is intended to be maintained in contact with metal surfaces for fairly long periods, as compared with ordinary removers which are now on the market.

Again, it will be noted that our paint remover is soluble in water and oil so that when it has loosened a protective coating from an article, it can readily be washed away with water, turpentine, petroleum naphtha, gasoline, or other readily available materials.

The water in the foregoing composition appears to have a very important function in that

it renders the penetrant solvents very active in attacking both baked and air-dried varnishes. Thus, we have found that the preferred composition is extremely active at ordinary temperatures, but that when the water is omitted the paint lifting action is very much slower and less effective. The exact amount of water which is to be employed is determined to some extent by the consistency which the final product is to have. We have found that the proportion indicated above forms a remover paste of high effectiveness, but we recognize that a somewhat stiffer paste may be desirable at times, or that a softer one may also be useful, and accordingly that the water content may be adjusted to give a product most nearly meeting the needs of individual cases.

The monoethanolamine of the composition is an alkaline reacting solvent which is particularly effective in removing paints and varnishes of the resin base type. Almost all aircraft varnishes, for example, are based upon glycerol phthalate, and are readily acted upon by the monoethanolamine, even after they have been hard baked. In some cases we have found that this ingredient may be replaced by diethanolamine or triethanolamine, both of which will form soaps with oleic acid to give a paste-like remover, but neither of these amines is quite as effective in penetrating paints and lacquers as is the monoethanolamine of the preferred composition.

The kerosene constituent of the composition may be replaced with Stoddard solvent or No. 2 furnace oil. Gasoline and painters naphtha may also be used as substitutes, but are not preferred because of their low boiling points and high vapor pressures.

Mono nitropropane ( $\text{CH}_3\text{CH}_2\text{CH}_2\text{NO}_2$ ) in the presence of water is an effective solvent for attacking baked resin varnishes as well as air-dried varnishes of the linseed oil, China-wood oil and soya bean oil types.

Oleic acid is an unsaturated fatty acid which, as has been indicated, reacts with the monoethanolamine constituent to form a soap; and that that soap acts as a carrier for the several paint and varnish penetrants.

Isopropyl alcohol is a secondary mono-hydric alcohol having very good solvent properties and the ability to act as a blending agent for bringing the other mentioned ingredients into solution. It may be replaced in the composition by other secondary alcohols such as secondary butyl or secondary amyl alcohol.

The preferred form of the invention having been described, what is claimed as new is:

1. A paint and varnish remover comprising a paste-like mixture of about 12 percent by weight of water, about 10 percent by weight of monoethanolamine, about 13 percent by weight of monoethanolamine oleate, about 10 percent by weight of kerosene, about 36 percent by weight of 1-nitropropane, and about 19 percent by weight of isopropyl alcohol.

2. A paint and varnish remover comprising a mixture of about 10 parts by weight of monoethanolamine, about 8 parts by weight of kerosene, about 30 parts by weight of mononitropropane, about 9 parts by weight of oleic acid, about 16 parts by weight of isopropyl alcohol, and water, in which the oleic acid reacts with some of the monoethanolamine to form a soap, and in which the water is present in sufficient quantity so that the final mixture is of paste-like character.

3. A paint and varnish remover comprising a

mixture of about 10 percent by volume of water, about 10 percent by volume of monoethanolamine, about 20 percent by volume of kerosene, about 30 percent by volume of mononitropropane, about 10 percent by volume of oleic acid, and about 20 percent by volume of isopropyl alcohol, in which said oleic acid reacts with a portion of said monoethanolamine to form a soap, and in which the mixture is of paste-like character which may be spread readily over painted surfaces and will adhere thereto.

4. A paint and varnish remover comprising a

10 mixture of about 10 parts by weight of an ethanolamine, about 8 parts by weight of kerosene, about 30 parts by weight of mononitropropane, about 9 parts by weight of oleic acid, about 16 parts by weight of isopropyl alcohol, and water, in which said oleic acid reacts with a portion of said ethanolamine to form a soap, and in which said water is present in sufficient quantity so that the final mixture is of paste-like character.

JOHN D. MORGAN.  
RUSSELL E. LOWE.